

Jan. 7, 1941.

G. W. WALLACE

2,227,951

PROCESS FOR CARBONIZING COAL

Filed Feb. 23, 1938

3 Sheets-Sheet 1



INVENTOR

*G. W. Wallace*

Jan. 7, 1941.

G. W. WALLACE

2,227,951

PROCESS FOR CARBONIZING COAL

Filed Feb. 23, 1938

3 Sheets-Sheet 2



INVENTOR

*G. W. Wallace*

Jan. 7, 1941.

G. W. WALLACE

2,227,951

## PROCESS FOR CARBONIZING COAL

Filed Feb. 23, 1938

3 Sheets-Sheet 3



FIG. 6.



FIG. 8.

FIG. 7.



FIG. 9.

**INVENTOR**

Guisalace

## UNITED STATES PATENT OFFICE

2,227,951

## PROCESS FOR CARBONIZING COAL

George W. Wallace, East St. Louis, Ill.

Application February 23, 1938, Serial No. 191,910

4 Claims. (Cl. 202—26)

This invention relates to the carbonization of coal and similar solid carbonaceous substances and its principal object is to provide an improved process of and apparatus for effecting the carbonization of coking or semi-coking coal and it is primarily adapted to carbonizing slack coal or screenings and more particularly adapted to carbonizing the fine coal and dust resulting from the preparation of so called stoker fuel where the product is often as fine as a minus ten mesh material.

Another object of the invention is the production of smokeless fuel by low temperature carbonization.

15 A further object of the invention is the production of a smokeless fuel under conditions wherein the volatile content of the resultant product may be controlled within close limits to that desired.

20 And still another object is the production of a low temperature smokeless fuel of improved structure and denseness.

Other objects and desirable features of the invention will be hereinafter pointed out.

In the present invention the process of carbonizing coal consists in causing the coal to pass through a carbonization chamber supported on a moving or movable pan or apron conveyor, regulating the depth of coal in the pans or thickness of layer on the apron to that desired and covering the coal in the pans or layer on the aprons with a series of covers of sufficient weight to affect the structure and compactness of the resultant fuel product and heating the coal undergoing carbonization from beneath the supporting medium and above the covers with hot gaseous products of combustion in direct contact with both the supporting medium and covers to effect the carbonization.

40 The hot gaseous products of combustion may be produced by burning gas with air and are preferably produced by burning the gases resulting from the operation of the process. The temperatures of the hot gaseous products of combustion are controlled by using an excess of gas where gases are burned with air to produce said hot gaseous products of combustion.

45 Figure 1 of the drawings is a vertical sectional view of one form of apparatus that can be used in practicing the present process. The section is taken on line 1—1 Fig. 2 and illustrates a pan type of conveyor or supporting medium.

Figure 2 is a section of the apparatus in plan taken on line 2—2 Fig. 1.

50 55 Figure 3 is a vertical section taken on line

3—3 Fig. 2 and illustrates the manner in which the links support the pans.

Figure 4 is a vertical cross section of the apparatus on line 4—4 Fig. 1 and illustrates the manner in which the hot combustion gases are admitted to the carbonization chamber.

Figure 5 is a vertical cross section of the apparatus on line 5—5 Fig. 1 and illustrates the manner in which the hot combustion gases leave the chamber.

10 Figure 6 is a broken vertical sectional view of another form of apparatus which can be used in practicing the present invention and illustrates one type of apron conveyor which may be used.

Figure 7 is a vertical section in part on line 15 1—1 Fig. 6.

Figure 8 is an enlarged view of the driving sprocket illustrating the manner in which the covers may be brought into position and placed on top of the coal.

20 Figure 9 is a cross section through line 9—9 Fig. 6 and illustrates a damper control of the hot gaseous products of combustion.

Said apparatus consists of, a carbonizing chamber constructed of refractory material A 25 which may be a lining within a sheet metal casting not shown, a conveyor or supporting medium B for the coal being carbonized which may consist either of shallow pans or an apron conveyor, a series of more or less loosely riding covers C 30 which are arranged to cover the coal in the pans or on the apron conveyor and which are of sufficient weight to affect the structure of the carbonized residue or smokeless fuel. The said supporting medium and covers may be constructed 35 of steel, cast steel, cast iron, or a special alloy of iron having heat resisting properties, usually two or more of such metals will be used in assembling the apparatus. A coal hopper D is provided from which the coal to be carbonized is 40 fed onto the pans or onto the apron conveyor at the desired depth or thickness. In the apparatus sprocket wheels E actuate the conveyor and sprocket wheels E' which are synchronized with sprockets E actuate the covers, tail sprockets F 45 and F' reverse the direction of the conveyor and covers to the point of loading. Links G carry the weight of the pans or aprons and in turn are supported by rods H which are connected with wheels I which travel on rails J, links G' carry 50 the covers excepting when they are resting on the coal and are supported by rods H' and wheels I' which travel on rails J'. A driving gear K, preferably of variable speed is provided to actuate the sprocket wheels E and E' said driving

20

30

40

50

60

70

80

90

100

110

120

130

140

150

160

170

180

190

200

210

220

230

240

250

260

270

280

290

300

310

320

330

340

350

360

370

380

390

400

410

420

430

440

450

460

470

480

490

500

510

520

530

540

550

gear may be powered in any suitable manner for instance by an electric motor K'. In the apparatus as illustrated means are provided for admitting hot products of combustion beneath the coal supporting medium and above the covers at L through a series of flues M below the supporting medium and through a series of flues M' above the covers. The hot gaseous products of combustion after passing through the flues M and M' leave the carbonization chamber at N from which they are conducted to the desired condensing and scrubbing apparatus not shown. The product of the carbonization or smokeless fuel is discharged from the conveyor or supporting medium into the hopper O from which it is removed from the carbonization chamber by means of star feeder P which serves also to prevent any air entering the chamber at this point. It is to be understood that the hopper O may be of any desired size. With certain coals it may be desirable to use the apron conveyor or supporting medium B Fig. 6 which provides means X for assisting in the removal of the carbonized residue from the supporting medium. In the apparatus R Fig. 1 is a refractory top and bottom for flues M and M' which if desired may be dispensed with. In Figs. 1 and 2 the flues M and M' are shown as cross flues which conduct the hot combustion gases back and forth across and beneath the supporting medium and above the covers from the inlet L as shown in Figs. 2 and 4 to the outlet N as shown in Figs. 2 and 5. Fig. 6 illustrates a single longitudinal open flue S beneath the supporting medium and S' above the covers, in this illustration the top and bottom refractory lining R as shown in Figs. 1, 4 and 5 is omitted. In order to control the hot combustion gases entering and leaving the open flues S and S' baffles T and T' may be provided at the inlet and outlet of said flues the baffles having a series of ports which may be adjusted by partially opening or closing dampers U and U' as shown in Fig. 9. By the use of these dampers the hot combustion gases entering the carbonization chamber beneath the supporting medium and above the covers at inlet L and leaving the chamber at outlet N may be distributed uniformly below and above the coal being carbonized.

While two different systems of flues have been illustrated other arrangements of passing the hot combustion gases used to effect the carbonization into and through the carbonization chamber, may be used and in some cases it may be desirable to effect the carbonization by passing the hot combustion gases beneath the supporting medium only, this would apply particularly to coal having unusual swelling and plastic characteristics. The hot gaseous products of combustion used to effect the carbonization are preferably admitted to the carbonization chamber at the discharge end of the coal supporting medium, and caused to pass in countercurrent to the direction of movement of the coal through the chamber, and removed from the end where the coal is fed onto the supporting medium.

In synchronising the placing of the covers on the coal short rails V Fig. 3 may be used to guide the covers as they leave sprockets E' and position them properly on the coal after which the full weight of the covers, links, rods and wheels will be on the coal body during the carbonization period until short guide rails V' pick the weight up as the covers reach sprocket wheels F', or the modification shown in Figs. 6 and 8 may be used in which case the covers are positioned over

the coal either on the pans or aprons of the conveyor directly from sprocket wheels E' which are synchronized with sprocket wheels E and as the supporting medium and covers move forward into the carbonization chamber the weight of the covers is transferred to the coal due to the slots W shown in Figs. 6, 7 and 8 moving up on rods H' freeing the covers from any support until they are lifted from the carbonized residue by sprocket wheels F'.

Other means of placing the covers on the body of coal being carbonized and properly synchronising the same with the body of coal on the supporting medium may be used, the drawings illustrating two practical methods.

The primary object of the covers is to compress the coal during carbonization particularly while it is passing through the plastic stage so as to produce as dense and compact a product as possible.

The coal or material to be carbonized may be passed through the carbonization chamber either continuously or intermittently, it may be advanced through the chamber for short distances at frequent intervals or through substantial distances with correspondingly long stationary periods between the intervals of movement. While the continuous movement of the material through the chamber is preferable the intermittent movement is entirely practical.

The hot gaseous products of combustion used to effect the carbonization are preferably produced entirely outside the carbonization chamber by burning gases with air the gases being in excess of the amount of air required for the theoretical complete combustion of the same. The temperature of the hot gaseous products of combustion is controlled by the amount of excess gas used, i. e., 60 parts of a 120 B. t. u. gas and 40 parts air will furnish products of combustion having a lower temperature than when using 50 parts gas and 50 parts air, by using this method of regulating the carbonization and controlling the temperature of the gaseous products of combustion used to effect the carbonization temperatures of 550°C. to 800°C. may be maintained uniformly, and higher or lower temperatures may be secured and controlled if desired, the greater the amount of excess gas used the lower is the temperature of the products of combustion. The hot gaseous products of combustion are preferably of a reducing nature as this condition serves to protect the mental portions of the apparatus. While a less desirable result would be secured it is possible to have the combustion of the gases take place partially within the carbonization chamber.

The gases resulting from the operation of the process are usually sufficient in amount and quality to furnish the hot gaseous products of combustion used to effect the carbonization. If for any reason it is not desirable to use the gases resulting from the operation of the process producer gas may be used or any other combustible gas or fuel or a furnace may be installed to furnish the hot gaseous products of combustion. If desired instead of using an excess of gas to control the temperature of the hot gaseous products of combustion the same may be controlled by admixing or diluting with inert gas and/or steam or the temperature may be controlled in any other suitable manner.

The thickness or depth of the body of coal or material to be carbonized may be regulated by gate Y attached to hopper D as shown in Figs. 75

1 and 6, the gate Y shown in Fig. 1 may if desired be arranged so as to bring the level of the coal in the pans to a point level with or just below the top of the pans, the gate Y as shown in Fig. 6 5 may be adjusted so as to control the thickness of the layer or body of coal to that desired.

The thickness of the layer or body of coal may vary considerably with different coals however a thickness of from three to four inches should 10 meet any usual requirements as relatively thin layers will carbonize more efficiently.

In practicing the process of the present invention a layer of coal of the desired thickness is fed from hopper D on to the moving or movable conveyor or supporting medium B which enters the carbonization chamber within A where the coal is covered and compressed by covers C. Hot gaseous products of combustion are passed beneath the supporting medium and above the covers to effect the carbonization of the coal at a 15 temperature of from 550° C. to 650° C. for low temperature carbonization where around 8 to 12% volatile matter is desired in the resultant fuel and at higher temperatures where a lower amount 20 of volatile matter is wanted. The rate at which the coal travels through the chamber is adjusted so that the carbonization is complete when the residue is discharged into hopper O from which it is removed through sealing device and feeder P 25 and from which point it is cooled and taken to storage.

The gases, oils and liquids distilled from the coal during carbonization escape around or through the covers which may be perforated if 30 desired and between the sections of the supporting medium and they are removed from the carbonization chamber entrained with the hot gaseous products of combustion. The combined gases may be cooled and washed in any manner desired 35 to remove such of the coal tar and other by-products as it may be found profitable or desirable to recover. An exhauster may be used to remove the gases and vapors from the carbonization chamber under a partial vacuum and deliver them 40 under pressure to the condensers or place of use. The amount of gas required to effect the carbonization may if desired be returned to a combustion chamber which may form a part of the carbonizing apparatus where it is burned with 45 air to produce the hot gaseous products of combustion, the temperature of said products being controlled and regulated in the manner described. The excess gas produced in the operation of the 50 process and not used for carbonization purposes may be used otherwise or may be wasted.

I claim:

1. The process of carbonizing coking coal to

produce a substantially smokeless fuel which consists in confining the coal in shallow pans, and continuously passing the paned coal in a substantially horizontal direction through a hot carbonizing chamber, the coal being confined across its upper surfaces by loosely riding covers of sufficient weight to produce a relatively small-pored dense coke while permitting escape of the gaseous products of such carbonization. 5

2. The process of carbonizing coking coal to 10 produce a substantially smokeless fuel which consists in confining the coal in shallow pans, and continuously passing the paned coal in a substantially horizontal direction through a hot carbonizing chamber, having a temperature range 15 from 550° C. to 800° C., the coal being confined across its upper surfaces by loosely riding covers of sufficient weight to produce a relatively small-pored dense coke while permitting escape of the 20 gaseous products of such carbonization.

3. The process of carbonizing coking coal to 25 produce a substantially smokeless fuel which consists in confining the coal in shallow pans, continuously passing the paned coal in a substantially horizontal direction through a carbonizing chamber, the coal being confined across its upper surfaces by loosely riding covers of sufficient weight to produce a relatively small-pored dense coke while permitting escape of the gaseous 30 products of such carbonization, and passing hot gaseous products of combustion through the chamber in a direction opposite to the direction of movement of the coal, said products of combustion being produced by burning combustible gases with 35 air in an amount insufficient for their complete combustion.

4. The process of carbonizing coking coal to 40 produce a substantially smokeless fuel which consists in confining the coal in shallow pans, continuously passing the paned coal in a substantially horizontal direction through a carbonizing chamber, the coal being confined across its upper surfaces by loosely riding covers of sufficient weight to produce a relatively small-pored dense coke while permitting escape of the gaseous 45 products of such carbonization in a serpentine path generally counter-current to the movement of the coal, and passing hot gaseous products of combustion through the chamber in a direction opposite to the direction of movement of the coal, said 50 products of combustion being produced by burning combustible gases with air in an amount insufficient for their complete combustion.

GEORGE W. WALLACE. 55